

Nov. 24, 1959

A. H. SOMMER

2,914,690

ELECTRON-EMITTING SURFACES AND METHODS OF MAKING THEM

Filed Dec. 5, 1955



INVENTOR.  
ALFRED H. SOMMER  
BY

William A. Zalewski  
ATTORNEY

# United States Patent Office

2,914,690

Patented Nov. 24, 1959

1

2,914,690

## ELECTRON-EMITTING SURFACES AND METHODS OF MAKING THEM

Alfred Hermann Sommer, Princeton, N.J., assignor to Radio Corporation of America, a corporation of Delaware

Application December 5, 1955, Serial No. 551,028

9 Claims. (Cl. 313—65)

This invention relates to electron discharge devices having films and to the art of making them, and, particularly, to electron-emitting films for use in phototubes, photomultiplier tubes, camera tubes for television and the like.

Electron-emitting films emit electrons when bombarded by visible or invisible radiation, charged particles, electrons or the like. Such films may be made by properly depositing and reacting a plurality of chemical substances on a support member of glass or metal or the like. One type of electron-emissive film emits electrons when bombarded by visible or invisible radiation and is known as a photocathode.

In general, a good photocathode film has high and uniform sensitivity, that is, the film emits the same large number of electrons from all areas thereof that are under identical light conditions. In some types of pickup tubes, the photocathode is planar and incident light strikes one surface and the photoelectrons are emitted from the opposite surface. Thus, the requirement is imposed that the film be thin enough to be penetrated and excited by the incident light. In order to replace emitted electrons, the cathode film is electrically connected to a source of electrons and another requirement is that the cathode film be sufficiently thick to have the requisite conductivity to achieve electron replacement. An optimum photocathode film is of uniform thickness so that electron emission and electron replacement are achieved uniformly over the entire area thereof. However, present methods of preparation do not provide such uniform photocathode film.

In the method of making a photocathode in accordance with this invention, a suitable support plate of glass, or the like, is first provided with a thin film of potassium and then an electron-emitting surface, such as a photocathode surface, is formed thereon. The electron-emitting surface may be an alkali-activated antimony system or the like. The thin potassium film promotes the formation of a uniform and sensitive photocathode which is comparatively easily reproduced.

In the drawing,

Fig. 1 is an elevational view partly in section of one type of electronic device embodying the principles of the invention;

Fig. 2 is an elevational view of a portion of the device shown in Fig. 1;

Fig. 3 is a sectional view along the line 3—3 in Fig. 2; and,

Fig. 4 is an enlarged sectional view of a portion of the face plate and photocathode in the tube shown in Fig. 1.

For purposes of illustration, the following description relates to a television camera pickup tube which utilizes an alkali-antimony photoemissive surface or photocathode made according to the principles of the invention. Referring to Fig. 1, a television camera tube 10, for example, of the image orthicon type, includes an envelope 12 having a face plate 14 on the inner surface of which a photoemissive surface or photocathode 16 is provided

2

according to the principles of the invention. Voltages are shown in Figure 1 for purposes of illustrating the operation of the tube. These voltage values are not limiting. In operation of the tube of Fig. 1, a scene which is to be televised is optically focused upon the face plate 14 and on the photocathode 16. Photoelectrons are released from the photocathode with a pattern of distribution corresponding to the pattern of light coming from the scene to be televised. The photoelectrons are focused upon a thin glass target 18 by an electromagnetic coil 20 which surrounds the envelope 12 and provides a uniform magnetic field coaxial therewith. The photoelectrons are also accelerated toward the glass target by ring electrodes 22 and 23 so that they strike the glass target 18 with sufficient energy to produce secondary emission therefrom. A fine mesh screen 24 is positioned closely adjacent to the surface of the target 20 and collects the secondary electrons. The loss of electrons from the surface of the glass target leaves a positive charge 20 pattern on the glass target surface corresponding in distribution in intensity to the optical scene focused on the photocathode 16. Since the glass target is very thin, a corresponding pattern of potentials is present on the surface away from the photocathode.

25 The last-mentioned surface of the glass target is scanned by an electron beam formed by an electron gun 26 located at the opposite end of the tube from the photocathode. The electron beam is aligned by oppositely disposed coils 25 and 25', and is focused on the target 18 by the coil 20. The beam is scanned over the surface of the target by deflection fields produced by coils formed into a yoke 27, and is well known in the art. As the electrons of the beam approach the target 20 they are decelerated to substantially zero velocity by 30 means of a decelerating ring electrode 28. Some of the electrons from the cathode ray beam are deposited on the positive areas of the target surface in an amount to neutralize the positive charges on the opposite surface of the target. These deposited electrons drive each positive 35 target area to gun cathode potential so that the remainder of the beam electrons are reflected back along the tube envelope toward the electron gun 26 by the neutralized target area. The reflected electrons are collected and amplified in a multiplier section 30 to form video signals 40 in the output circuit of the tube (not shown).

Electrical connection is made to the photocathode 16 by means of a strip of silver 32 (Fig. 2) painted on the inner wall of the envelope 12 in contact with the photocathode 16. A spring contact lead 34 contacts the silver strip and is connected, as by welding, to a pin 36 which extends through the wall of the envelope and to which electrical contact may be made. Similarly, the accelerating electrodes 22 and 23 are welded to wire leads 37 and 38, respectively, which extend through the wall 55 of the envelope.

A heater filament 40 of tungsten or the like, for use in evaporating material during the making of the photocathode 16, is disposed between the mesh screen 24 and the electrode 23 as shown in Fig. 3. One end of the filament is secured to a lead 42 which passes insulatingly through the electrode 23 and is welded to a pin 43 which extends through the wall of the envelope. The other end of the filament 40 is secured to the electrode 23 by a lead 44. Thus, electrical connection to the filament is provided through the external pins 38 and 43. Three other chemical carriers 45, 46 and 47 (Fig. 3), each in the form of different elongated metal channels, as shown, or in any other convenient form, are also provided within the envelope 12. In one convenient arrangement, one 60 end of each carrier 45, 46 and 47 is secured to the outer surface of accelerating electrode 23 and the other end of each carrier is secured to wire leads 48, 49 and 50, re-

spectively, which extend through the wall of the envelope. Thus, external electrical connections are provided for passing current through each of the chemical carriers 45, 46 and 47.

In assembling the tube, the materials to be evaporated are prepared as pellets, powders or the like and are secured to or deposited in their various carriers or support members. Specifically, a plurality of pellets or beads 52 comprising high grade commercial antimony with only traces of iron, sulfur, arsenic and lead permitted are secured, at spaced intervals, on the filament 40. A mixture of one part by weight of potassium chromate, one part by weight of aluminum, and 8 parts by weight of tungsten is placed in the carrier 45. A mixture of one part by weight of sodium chromate, one part by weight of aluminum and 8 parts by weight of tungsten is placed in the carrier 46. A mixture of one part by weight of cesium chromate and 3 parts by weight of silicon is placed in the carrier 47. The percentages of the various components of the latter three mixtures disposed in the carriers 45, 46 and 47 are not critical and may be varied within wide ranges, as desired.

After the various tube components are assembled in the envelope 12, the tube is mounted on an exhaust pump by means of an exhaust tubulation (not shown) and then baked at a temperature in the range of 375° to 400° C. for about one hour to remove occluded gases from the envelope and from the metal parts.

The photocathode film 16 is prepared in the following manner: First, the tube is heated, for example in an oven, to a temperature in the range of 140° C. to 170° C. With the tube thus heated, a thin film 54 (Fig. 4) of potassium is evaporated onto the inner surface of the face plate 14 of the envelope 12. This evaporation is effected by passing current from a suitable power source (not shown) through the leads 38 and 48 and heating the carrier 45 and thereby evaporating potassium metal released by the reaction of the potassium chromate, aluminum and tungsten. As the potassium is deposited on the face plate the photoelectron emission therefrom is measured and when the emission reaches a peak value, the evaporation of potassium is discontinued.

This electron emission from the potassium film may be measured by connecting the photocathode by its lead 36 and the electrode 23 by its lead 38 in series with an ammeter 56 and then directing light from a source 58 onto the face plate. The tube is kept at an elevated temperature as described above to render the glass of the face plate conductive so that the foregoing measurement of the potassium film may be made during the evaporation of the potassium. The potassium film thus formed is invisible and is believed to be in the form of a monatomic layer.

Next, a film 60 of antimony is deposited over the potassium film 54 on the face plate 14. This operation may be performed with the tube at room temperature. In order to evaporate the antimony from the pellets 52 a heating current is passed through the leads 38 and 43 to heat the filament 40 to the vaporization temperature for the antimony metal. For reasons which are not fully understood, the presence of the potassium film on the face plate promotes the formation of a thinner, more uniform antimony film than would be formed on the glass face plate alone. The deposition of the antimony may be continued until the light transmission from the source 58 through the face plate is in the range of 50 percent to 95 percent of the light passed prior to the formation of the film. The light transmission through the face plate may be measured by means of a photocell in the manner disclosed in U.S. Patent No. 2,676,282 of J. J. Polkosky. The light transmission prior to the deposition of the film may be arbitrarily assumed to be 100.

To form one type of photocathode, the antimony film 60 is then activated with three alkali metals, potassium,

sodium, and cesium. First, the tube is again heated to a temperature in the range of 140° C. to 170° C. in order to control the amount of potassium deposited on the film 60. Potassium is then evaporated onto the antimony film from the material remaining in the carrier 45 by passing heating current therethrough by way of the pins 38 and 48. The evaporation of the potassium is continued until the photo-emission reaches a peak value as indicated by ammeter 56. Evaporation of potassium is then discontinued and the temperature of the tube is raised to about 220° C. and the excess potassium metal is pumped out.

The tube is then held at a temperature in the range of 180° C. to 220° C. and the antimony film is treated with a second alkali metal, sodium, which is evaporated onto the coated face plate by heating and reacting the material in the carrier 46. The requisite heating may be achieved by passing current through the leads 38 and 49. The evaporation of sodium is also continued until peak photoemission is achieved and the excess is then pumped out of the tube.

Finally, the tube temperature is brought into the range of 130° C. to 160° C. and cesium is evaporated onto the coated face plate from the carrier 47 until electron emission from the photocathode reaches a peak value and the excess cesium is pumped out. Thus, the photocathode 16 is essentially complete and the tube is cooled and processed further as required.

Under some circumstances, it may be desirable to evaporate additional antimony onto the photocathode, as it is formed, after each activation with an alkali metal.

In the foregoing process, the order in which the sodium and potassium are evaporated onto the antimony coated face plate may be reversed. In addition, the principles of the invention may also be employed with secondary electron-emissive coatings and with other photocathode systems, for example, antimony-potassium-rubidium, antimony-rubidium-potassium, antimony-potassium-sodium, antimony-sodium-potassium, antimony-potassium-lithium or the like. In each case, the selected photocathode system is formed on a face plate coated with a film of potassium.

The method of the invention provides electron emitting surfaces which exhibit sensitivities over their areas which do not vary by more than about 3 percent to 7 percent. For example, one photocathode showed sensitivities varying over the whole surface in the range of 170 to 175 microamperes per lumen of incident light. On the other hand, photocathodes made according to prior art practices have sensitivities over their areas which may vary up to 90 percent. For example, one such photocathode had sensitivities in the range of 20 to 110 microamperes per lumen.

Thus, the method of the invention provides electron-emitting surfaces which are reproducible and which have high and uniform sensitivity.

What is claimed is:

1. An electron-emissive electrode comprising a supporting base, a film of potassium on said base, a film of antimony on said potassium film, said antimony film including reaction products of antimony with a plurality of alkali metals.
2. An electron-emissive electrode comprising a supporting base, a film of potassium on said base, a film of antimony on said potassium film, said antimony film including reaction products of antimony with sodium and potassium.
3. An electron-emissive electrode comprising a supporting base, a film of potassium on said base, a film of antimony on said potassium film, said antimony film including reaction products of antimony with sodium, potassium and cesium.
4. An electron-emissive electrode comprising a supporting base, a film of potassium on said base, a film

of antimony on said potassium film, said film including small amounts of a plurality of alkali metals.

5. An electron-emissive electrode comprising a supporting base, a film of potassium on said base, a film of antimony on said potassium film, said film including small amounts of sodium, potassium and cesium.

6. An electron-emissive electrode comprising a supporting glass base, a film of potassium on said base, a film of antimony on said potassium film, said film including small amounts of potassium and lithium.

7. An electron-emissive electrode comprising a supporting glass base, a film of potassium on said base, a film of antimony on said potassium film, said film including small amounts of at least two alkali metals.

8. An electron discharge device including an electron-emitting portion, said portion comprising a supporting base, a film of potassium on said base, a film of antimony on said potassium film, said antimony film including re-

action products of antimony with a plurality of alkali metals.

9. A camera tube comprising an envelope, a face plate at one portion of said envelope, an electron-emissive surface on said face plate and including a film of potassium on said face plate, and a film of antimony on said film of potassium, said film of antimony including reaction products of antimony with a plurality of alkali metals.

10

References Cited in the file of this patent

UNITED STATES PATENTS

|           |         |                |
|-----------|---------|----------------|
| 2,206,372 | Sommer  | July 2, 1940   |
| 2,391,280 | Teal    | Dec. 18, 1945  |
| 2,603,757 | Sheldon | July 15, 1952  |
| 2,654,048 | McGee   | Sept. 29, 1953 |
| 2,747,133 | Weimer  | May 22, 1956   |
| 2,770,561 | Sommer  | Nov. 13, 1956  |